# EUROPEAN PATENT SPECIFICATION

(11) **EP 2 069 266 B1**
(45) Date of publication and mention of the grant of the patent: **05.03.2014**
(21) Application number: 07826235.9
(22) Date of filing: 03.09.2007
(51) Int. Cl.: C06B 31/28, C06B 47/00

(54) **Process for the production of an explosive**
Verfahren zur Herstellung eines Sprengstoffs
Procédé de fabrication d'un explosif

(30) Priority: 04.09.2006 ZA 200607393
(43) Date of publication of application: 17.06.2009
(73) Proprietor: AEL MINING SERVICES LIMITED, Woodmead 2196 Gauteng (ZA)
(72) Inventor: TYLER, Dave, Alfred, Mufulita (ZM); VERMAAK, Charl, 2158 Johannesburg (ZA); ANTHONY, Derek, Luke, 1609 Edenvale (ZA)
(74) Representative: Gill, Siân Victoria
(86) International application number: PCT/IB2007/053534
(87) International publication number: WO 2008/029339

(56) References cited:
- EP-A- 0 318 424
- WO-A-97/30955
- GB-A- 882 665
- US-A- 3 095 335
- US-A- 4 775 431
- US-A- 5 397 405
- US-A- 5 486 247
- US-A1- 2003 029 346
- CHEMICAL ABSTRACTS, vol. 133, no. 21, 20 November 2000 (2000-11-20), Columbus, Ohio, US; abstract no.: 298420m, T.C. RUHE ET AL.: "Thermal stability of ANFO made with recycled oil" XP002500465 & Proc. Annu. Conf. Explos. Blasting Tech. 1999, 25th (Vol. 2), pages 263-271, International Society of Explosive Engineers

## Description

THIS INVENTION relates broadly to ammonium nitrate/fuel oil explosive, also known as ANFO explosive, and hereinafter referred to as ANFO explosive. More particularly, the invention relates to a process for producing an ANFO explosive, and to an ANFO explosive when produced in accordance with the process.

A process for producing an ammonium fuel oil (ANFO) explosive, wherein an emulsion comprising diesel fuel oil and water is mixed with ammonium nitrate prills is described in US Patent no. 4,775,431.

According to the invention, broadly, there is provided a process for producing an ammonium nitrate fuel oil (ANFO) explosive, the process including:
admixing used lubricating oil with water in the absence of any virgin oil to form a fuel consisting of a water-in-oil emulsion; and
admixing the emulsion with solid particulate ammonium nitrate to absorb the emulsion into the ammonium nitrate to form an ANFO explosive.

More particularly, the lubricating oil may be of the type employed for the lubrication of motor vehicles, such as utility vehicles of the kind used in mines, or for the lubrication of similar machinery. The particulate ammonium nitrate in turn will typically be in the form of porous prills of the type conventionally used for the manufacture of ANFO explosives.

The relative proportions of emulsion and ammonium nitrate employed will be more or less conventional, such that, in the product ANFO explosive, the oil forms 5-8% by mass, typically 5-7% by mass, e.g. 6% thereof. In the emulsion, the oil may form 55-86% by mass, preferably 72-78% by mass, e.g. 75% thereof. The balance is thus naturally water. Thus, when the oil forms 75% by mass of the emulsion, water forms 25% by mass thereof.

Admixing the oil with the water to form the emulsion may be by means of high-shear mixing, eg by using a high-shear mixer. The admixing may be effected in the presence of a suitable emulsifier/surfactant, which may form 0.2-1.0% by mass of the emulsion, preferably 0.3-0.8%, e.g. 0.5% thereof.

While all of the emulsifier/surfactant can be added to the oil, to the water and/or to an oil/water mixture, at least a portion of the emulsifier/surfactant may already be present in the oil, so that, at most, only any shortfall in the emulsifier/surfactant is then added to the oil, to the water or to the oil/water mixture.

Admixing the emulsion with the porous prilled ammonium nitrate (PPAN) may be in conventional fashion by pumping the emulsion from a source tank and spraying it by means of a nozzle on to the ammonium nitrate which is moved along by the flutes of an auger to provide additional mixing. To prepare the ANFO explosive on a batch scale, a concrete mixer or the like may be used. A PPAN:fuel ratio of 95:5-85:15, preferably 94:6-91:9, e.g. 92:8, may be used.

The invention extends also to an ANFO explosive when produced in accordance with the process described herein.

The invention will now be described, by way of example, with reference to the accompanying non-limiting illustrative worked Example.

### EXAMPLE

Mine utility vehicle waste lubricating oil was mixed in a high-shear mixer with water using an emulsifier/surfactant, to form a water-in-oil emulsion. The mixer used was an off-the-shelf mixer marketed under the trade designation Jones Industrial Mixer by Jones Process Equipment as manufacturer; and the emulsifier/surfactant used was an off-the-shelf sorbiton monooleate made by Croda Chemicals (SA) (Pty) Limited, 4 Covora Street, Jet Park, PO Box 1642, 1620 Kempton Park, South Africa. After mixing the oil and water into a stable homogeneous emulsion, comprising 0.5% by mass emulsifier/surfactant, 24.5% by mass water and 75% by mass oil, the emulsion was admixed with PPAN by pumping the emulsion from a source tank and spraying it by means of a nozzle on to the ammonium nitrate prills which were moved along by the flutes of an auger to provide additional mixing, to cause absorption of the emulsion into the PPAN, in a PPAN:emulsion mass ratio of 92:8. The emulsion was found to be absorbed almost immediately into the PPAN to form an ANFO explosive.

The ANFO explosive was subjected to detonation tests in comparison with standard ANFO explosive made from PPAN and a fuel comprising Shellsol 2325 (trademark) mining solvent, and was found to behave in comparable fashion as far as plate detonation tests and velocity of detonation (VOD) were concerned.

The Applicant is aware that used mine utility vehicle oil, which is generated in large volumes, has been used in the past for the manufacture of ANFO explosive. For example, the use of recycled (used) lubricating oil from mining equipment for the manufacture of ANFO explosives is known from T.C. Ruhe et al.: "Thermal stability of ANFO made with recycled oil" published in Proc. Annu. Conf. Explos. Blasting Tech. 1999, 25th (Vol. 2), pages 263-271, International Society of Explosive Engineers. However, it is refractory and difficult to absorb into PPAN by itself, so that it must be diluted with diesel or other virgin oil, such as the mining solvent available in South Africa under the trade mark Shellsol 2325 from Shell South Africa Energy (Pty) Limited of Shell Court, 33 Baker Street, Rosebank 2196, PO Box 747, Saxonwold 2132, South Africa. When the ANFO explosive comprises, as is typically the case, 5-7% by mass fuel oil, the balance being PPAN, no more than about 2-3% of the ANFO explosive can be waste mine utility vehicle oil, the remaining 3-4% being required to be virgin diesel or Shellsol. This is a disadvantage, because of the cost of the virgin oil, and because of the lowered consumption of used or waste oil. It is thus a particular advantage of the present invention that it obviates the use of any virgin oil to dilute the waste oil, the virgin oil being supplanted by water and economically attractive small amounts of emulsifier/surfactant. Disposal in this fashion of the waste oil is thus ecologically desirable and economically attractive.

## Claims

1. A process for producing an ammonium nitrate fuel oil (ANFO) explosive, the process including:
admixing used lubricating oil with water in the absence of any virgin oil to form a fuel consisting of a water-in-oil emulsion; and
admixing the emulsion with solid particulate ammonium nitrate to absorb the emulsion into the ammonium nitrate to form an ANFO explosive.

2. A process according to Claim 1, wherein the used lubricating oil is that obtained from mining vehicles.

3. A process according to Claim 1 or Claim 2, wherein the solid particulate ammonium nitrate is in the form of porous prills.

4. A process according to any one of Claims 1 to 3 inclusive, wherein the relative proportions of emulsion and ammonium nitrate employed are such that, in the ANFO explosive, the oil forms 5-8% by mass thereof.

5. A process according to any one of Claims 1 to 4 inclusive wherein, in the emulsion, the oil forms 55-86% by mass thereof.

6. A process according to any one of Claims 1 to 5 inclusive, wherein high-shear mixing is used to effect the admixing of the oil with the water to form the emulsion.

7. A process according to any one of Claims 1 to 6 inclusive, wherein the admixing of the used lubricating oil with the water to form the emulsion, is effected in the presence of an emulsifier/surfactant.

8. A process according to Claim 7, wherein the emulsifier/surfactant forms 0.2-1.0% by mass of the emulsion.

9. A process according to Claim 8, wherein the emulsion/surfactant forms 0.3-0.8% by mass of the emulsion.

10. A process according to any one of Claims 1 to 9 inclusive, wherein the admixing of the emulsion with the particulate ammonium nitrate is by pumping the emulsion from a source tank and spraying it by means of a nozzle on to the particulate ammonium nitrate which is moved along by the flutes of an auger to provide additional mixing, in an ammonium nitrate:emulsion ratio of 95:5-85:15.

## Patentansprüche

1. Ein Verfahren zur Herstellung eines Ammoniumnitrat-Brennöl (ANFO) Sprengstoffes, wobei das Verfahren
das Vermischen von gebrauchten Schmieröl mit Wasser in der Abwesenheit von nativem Öl, um einen Brennstoff bestehend aus einer Wasser-in-Öl Emulsion zu bilden, und
das Vermischen der Emulsion mit festem teilchenförmigen Ammoniumnitrat, um die Emulsion in das Ammoniumnitrat aufnehmen, um einen ANFO Sprengstoff zu bilden,
umfasst.

2. Ein Verfahren gemäß Anspruch 1, wobei das gebrauchte Schmieröl Schmieröl ist, das aus einem Bergbaufahrzeug erhalten wurde.

3. Ein Verfahren gemäß Anspruch 1 oder 2, wobei das feste teilchenförmige Ammoniumnitrat in Form von porösen Prills vorliegt.

4. Ein Verfahren gemäß einem der Ansprüche 1 bis einschließlich 3, wobei die relativen Anteil der Emulsion und des Ammoniumnitrats so eingesetzt werden, dass das Öl im ANFO Sprengstoff einen Anteil von 5 bis 8 Gewichts-% an diesem ausmacht.

5. Ein Verfahren gemäß einem der Ansprüche 1 bis einschließlich 4, wobei das Öl in der Emulsion einen Anteil von 55 bis 86 Gewichts-% an dieser ausmacht.

6. Ein Verfahren gemäß einem der Ansprüche 1 bis einschließlich 5, wobei Hochscher-Mischen verwendet wird, um das Vermischen des Öls mit dem Wasser zu bewirken, um die Emulsion zu bilden.

7. Ein Verfahren gemäß einem der Ansprüche 1 bis einschließlich 6, wobei das Vermischen des gebrauchten Schmieröls mit dem Wasser in Anwesenheit von einem Emulgator/einem Tensid bewirkt wird, um die Emulsion zu bilden.

8. Ein Verfahren gemäß Anspruch 7, wobei der Emulgator/das Tensid einen Anteil von 0.2 bis 1.0 Gewichts-% der Emulsion ausmacht.

9. Ein Verfahren gemäß Anspruch 8, wobei der Emulgator/das Tensid einen Anteil von 0.3 bis 0.8 Gewichts-% der Emulsion ausmacht.

10. Ein Verfahren gemäß einem der Ansprüche 1 bis einschließlich 9, wobei das Vermischen der Emulsion mit dem teilchenförmigen Ammoniumnitrat durch Pumpen der Emulsion aus einem Quellbehälter und Sprühen mithilfe einer Düse auf das teilchenförmige Ammoniumnitrat bewirkt wird, das weiterbewegt wird durch die Rillen einer Förderschnecke, um zusätzliches Vermischen zu bewirken, in einem Verhältnis von Ammoniumnitrat zu Emulsion von 95:5 bis 85:15.

## Revendications

1. Procédé de production d'un mélange explosif de nitrate d'ammonium et de fioul (ANFO), le procédé comprenant :
le mélange d'huile de graissage usagée et d'eau en l'absence d'une huile vierge quelconque pour former un combustible se composant d'une émulsion d'eau dans l'huile ; et
le mélange de l'émulsion et du nitrate d'ammonium particulaire solide pour absorber l'émulsion dans le nitrate d'ammonium pour former un explosif ANFO.

2. Procédé selon la revendication 1, dans lequel l'huile de graissage usagée est celle obtenue à partir de véhicules miniers.

3. Procédé selon la revendication 1 ou 2, dans lequel le nitrate d'ammonium particulaire solide se présente sous forme de granulés poreux.

4. Procédé selon l'une quelconque des revendications 1 à 3 inclus, dans lequel les proportions relatives d'émulsion et de nitrate d'ammonium utilisées sont telles que, dans l'explosif ANFO, l'huile constitue de 5 à 8 % en masse de celui-ci.

5. Procédé selon l'une quelconque des revendications 1 à 4 inclus dans lequel, dans l'émulsion, l'huile constitue de 55 à 86 % en masse de celui-ci.

6. Procédé selon l'une quelconque des revendications 1 à 5 inclus, dans lequel un mélange à cisaillement élevé est utilisé pour réaliser le mélange de l'huile et d'eau pour former l'émulsion.

7. Procédé selon l'une quelconque des revendications 1 à 6 inclus, dans lequel le mélange de l'huile de graissage usagée et d'eau pour former l'émulsion est réalisé en présence d'un émulsifiant/tensioactif.

8. Procédé selon la revendication 7, dans lequel l'émulsifiant/tensioactif constitue de 0,2 à 1,0 % en masse de l'émulsion.

9. Procédé selon la revendication 8, dans lequel l'émulsion/tensioactif constitue de 0,3 à 0,8 % en masse de l'émulsion.

10. Procédé selon l'une quelconque des revendications 1 à 9 inclus, dans lequel le mélange de l'émulsion et de nitrate d'ammonium particulaire est réalisé par pompage de l'émulsion à partir d'un réservoir source et par pulvérisation de celle-ci au moyen d'une buse sur le nitrate d'ammonium particulaire qui est déplacé le long des flûtes d'une tarière pour fournir un mélange supplémentaire, selon un rapport de nitrate d'ammonium/émulsion allant de 95/5 à 85/15.
